

## UNITED STATES PATENT OFFICE

ARCHIBALD JOHN HALL, OF CONGLETON, ENGLAND, ASSIGNOR TO THE SILVER SPRINGS BLEACHING & DYEING COMPANY LIMITED, OF CONGLETON, ENGLAND

## PROCESS FOR DYEING CELLULOSE ACETATE SILK IN FAST BLACK SHADES

No Drawing. Application filed August 26, 1929, Serial No. 388,635, and in Great Britain October 2, 1928.

This invention relates to the dyeing of black shades of exceptional fastness on cellulose acetate silk.

I have discovered, and this discovery forms the basis of this invention, that when cellulose acetate silk treated with solutions or colloidal dispersions of alpha-naphthylamine so as to absorb the alpha-naphthylamine is afterwards treated with solutions containing nitrous acid, the silk develops a deep black shade which has outstanding fastness to light, washing, rubbing, acids, alkalis, oxidizing and reducing agents.

I am aware that black shades may be produced on cellulose acetate silk by dyeing it with a suitable amino compound and then diazotizing with nitrous acid and coupling with a suitable naphthol such as beta-oxy-naphthoic acid, but my invention differs entirely from such methods and the black resulting from our invention is much faster and cheaper to produce.

The action of nitrous acid on cellulose acetate silk containing alpha-naphthylamine is largely dependent on the concentration, acidity, and temperature of the nitrous acid solution. Under certain conditions, particularly when the concentration of the nitrous acid is very small or the acidity of the solution is low, a brownish black shade results. But provided suitable conditions are employed the resulting black shade has a very pleasing tone.

I find that a satisfactory black shade is produced when the action of the nitrous acid is nearly complete in from 5 to 10 minutes but it is to be understood that the length of time in which the cellulose acetate silk should be immersed in the nitrous acid solution and/or the strength of such solution depends upon the nature of the cellulose acetate silk material. Thus in the case of yarn, a yarn having more twist will require a stronger solution if it is to penetrate the yarn in the same time as a yarn having less twist or if the same concentration is employed the penetration will require a longer time. Similar in a woven or knitted fabric the strength of the nitrous acid solution and/or the length of time for penetration

will depend both on the twist of the yarn and the closeness of the weave or knit.

The following example illustrates the invention but it is to be clearly understood that the conditions stated therein are by way of illustration only and are not intended to limit the method for applying my invention:

## Example

One gram of alpha-naphthylamine is dissolved in 5 grams of warm oleic acid and the resulting solution diluted with 150 c. c. of warm water containing a small amount of ammonia. Five grams of cellulose acetate silk are immersed in this solution at a temperature of 75° C. for one hour, then thoroughly washed with warm water, and immersed for 5 to 10 minutes in 150 c. c. of a solution at a temperature of 35-40° C., containing 1 gram of sodium nitrite and 5 grams of sulphuric acid per 100 c. c. The cellulose acetate silk thereby acquires a deep black shade and is afterwards, rinsed, soaped, rinsed and dried.

It is believed that the black pigment formed within the cellulose acetate fibres by the process hereinbefore described has the character of an oxidation product of alpha-naphthylamine in which a number of naphthalene residues are linked together by means of imino groups.

What I claim as my invention and desire to protect by Letters Patent is:—

1. Process for producing black shades on cellulose acetate silk which consists in first treating the cellulose acetate silk with alpha-naphthylamine so that the latter will be absorbed by the silk and subsequently treating the silk with nitrous acid for the development of a black shade thereon.

2. Process for producing black shades on cellulose acetate silk which consists in first treating the cellulose acetate silk with colloidal dispersions of alpha-naphthylamine so that the latter will be absorbed by the silk and subsequently treating the silk with nitrous acid for the development of a black shade thereon.

3. Process for treating cellulose acetate silk containing absorbed alpha-naphthyl-

amine by treating it with nitrous acid so as to produce black shades thereon.

4. Cellulose acetate silk having produced thereon a black shade comprising the oxidation product of alpha-naphthylamine with nitrous acid.

5. Process for producing black shades on cellulose acetate silk which consists in forming an oxidation product of alpha-naphthylamine within the cellulose acetate fibres by the action of nitrous acid on alpha-naphthylamine.

In testimony whereof I have hereunto set my hand, this 15th day of August, 1929.

15 ARCHIBALD JOHN HALL.

20

25

30

35

40

45

50

55

60

65